

## UNITED STATES PATENT OFFICE

2,546,941

## LUBRICATING OIL

William Davey, London, England, assignor to  
Shell Development Company, San Francisco,  
Calif., a corporation of Delaware

No Drawing. Application June 2, 1947, Serial No.  
751,993. In Great Britain July 25, 1946

15 Claims. (Cl. 252—48.4)

1

This invention relates to extreme pressure lubricants capable of withstanding high pressures at elevated temperatures under severe and adverse operating conditions. More specifically this invention pertains to improvement of extreme pressure lubricants by enhancing their extreme pressure properties and at the same time rendering them substantially non-corrosive and stable, by addition of a novel additive thereto, in rather minor amounts.

Natural and/or synthetic lubricants per se are not capable of withstanding extreme pressures at high temperatures, high speeds and under severe loading conditions as generally encountered in present day lubricating such as internal combustion engines of various types, transmission devices, certain types of gears, e. g. hypoid gears, metal fabrication such as in cutting and drawing and the like. Under such conditions of lubrication, the protective film formed between contacting surfaces, by the lubricant, so as to prevent direct metal-to-metal contact, breaks down or ruptures, and seizure or even welding of metal parts occurs, resulting in serious damage to the elements being lubricated. To overcome this serious weakness generally inherent in undoped lubricants, extreme pressure agents are added which form protective films between contacting surfaces and which possess among their properties the function of imparting film strength and oiliness to lubricants, thus preventing their breakdown and rupture under the above described lubricating conditions.

The action of extreme pressure agents is largely a physico-chemical phenomena and this accounts primarily for their effectiveness as extreme pressure agents. These agents or materials in addition to increasing the film strength of lubricants, become reactive with contacting surfaces forming thereon an alloying protective coating or film of great strength and thermal stability. This tenaciously adhering adsorbed protective film not only reduces friction between relatively movable parts such as encountered in internal combustion engines but also acts as an impermeable film which prevents corrosive acids and other contaminants from attacking the metal surface and the like. To be effective therefore extreme pressure must to a degree be reactive with contacting surfaces and form thereon a protective film which prevents welding of moving parts and aids lubrication. Since the reaction is normally between the additives in the lubricant and contacting surfaces at elevated temperatures of around about 500° C. and higher,

2

the performance of a given lubricant must depend upon its composition, the composition of the contacting surface being lubricated, as well as the conditions to which the combination is subjected.

Although extreme pressure additives to be effective should be reactive with contacting surfaces, this reactivity should not be corrosive to the reactive surface. This is generally a serious 10 drawback of known extreme pressure agents, for serious damage to surfaces such as alloy bearings and the like might result. Such additive should also not tend to promote oxidation which generally prompts formation of corrosive 15 acidic materials, sludge, lacquer and varnish which results in sticking and fouling of movable engine parts and the like.

Numerous compounds and mixtures of compounds have been tried as extreme pressure 20 agents for lubricants, the best of which have only moderately improved the extreme pressure properties of the lubricant and generally at the expense of increased corrosiveness and instability of the lubricant. Among such compounds 25 may be mentioned organic oxygen containing compounds such as fatty acids, esters, ketones, oxidized petroleum fractions; organic compounds containing sulfur or oxygen and sulfur such as sulfurized fatty oils, acids, etc.; organic compounds containing chlorine usually obtained by 30 chlorinating organic compounds or petroleum fractions; organic compounds containing phosphorus; organic compounds containing lead and especially such compounds when in conjunction with an active sulfur compound.

35 Of the general classes of extreme pressure compounds enumerated sulfur and/or halogen-containing compounds appear to be most effective and are therefore preferred. However these have serious defects in that most sulfur compounds to be effective must contain a major amount of sulfur in an active state which is highly corrosive and has a tendency of separating out and forms sludge. Materials of this type when in 40 combination with halogen-containing compounds have a deleterious effect by liberating highly corrosive acids from the halogenated compounds and also interfere with their functioning as an extreme pressure dope. Halogen-containing compounds, alone, become highly corrosive to alloy metals such as cadmium-silver, copper-lead, etc. so as to render them useless after short periods 45 of use.

50 It is an object of the present invention to provide an improved extreme pressure type lubri-

cant capable of effective lubrication under high pressures at elevated temperatures and adverse operating conditions. Still another object of this invention is to provide an improved, stable, sludge free, non-corrosive extreme pressure lubricant. Also it is an object of this invention to provide an improved extreme pressure lubricant by addition to any lubricating carrier or base a minor amount of a novel reaction product of this invention. Still another object is to form an improved non-corrosive extreme pressure additive from the reaction products of this invention. Other objects of this invention will appear as the description proceeds.

To the accomplishment of the foregoing and related ends, this invention consists of features which will be hereinafter fully described and particularly pointed out in the claims, the following description setting forth in detail certain embodiments of the invention, these being illustrative of but a few variations in which the principle of the invention may be employed.

Broadly stated, this invention is directed to the use in lubricants and the like, reaction products obtained by reacting a polyhalogen containing organic carbonyl compound with alkyl, aryalkyl, aryl, cyclic thiols, selenols, and/or telurols represented by the SH, SeH and TeH radicals respectively, the reaction being controlled so that the carbonyl radical reacts with the SH, SeH and/or TeH groups to form polyhalogenated thiol acetals, selenol acetals and/or telurol acetals, represented by the formula:



wherein R and R<sub>1</sub> represent the same or different radicals attached to the respective S, Se and/or Te atoms, represented by X, through a carbon linkage, as for example alkyl, aralkyl, aryl radicals which may contain substituents such as halogen, carboxylic acid groups, mercapto groups, thio ether groups, etc.; and the two other bonds terminating from the carbon atom having attached thereto at least one organic radical having a plurality of halogen atoms and from the other bond hydrogen or both of these bonds may have attached thereto organic radical having a plurality of halogen atoms. The position of the halogen atoms should be preferably such that they are as far removed from the carbonyl group as possible preferably on the end carbon atoms in relation to the position of the carbonyl group.

The polyhalogenated organic carbonyl compound may be polyhalogenated ketones or aldehydes. The following specific polyhalogenated organic carbonyl compounds which when reacted with thiol, selenol and/or telurol alcohols to form reaction products of this invention are:

I. Polyhalogenated aliphatic ketones of—acetone, methyl acetone, methyl isobutyl ketone, methyl n-butyl ketone, methyl n-amyl ketone, methyl isoamyl ketone, dipropyl ketone, methyl amyl ketone, ethyl amyl ketone, diisobutyl ketone, dibutyl ketone, methyl propyl ketone, diethyl ketone, 3-methyl heptanone, methyl vinyl ketone, pentanedione, pentanone, palmitone, laurone, stearone, pentadecanone, etc.

II. Polyhalogenated aromatic ketones of—acetophenone, benzophenone, benzyl phenyl ketone, dibenzyl ketone, etc.

III. Polyhalogenated cyclic ketones of—mesityl oxide, isophorone, cyclobutanone, cyclopentanone,

cyclohexanone, methyl cyclohexanone, methone, camphor, beta decalone, pulegone, piperitone, eucarvone, carvone, pino carvone, carvenone, etc.

IV. Other types of polyhalogenated ketones such as—diacetyl, acetylacetone, acetonylacetone, cyclohexandione, quinone, benzoylacetone, etc.

V. Polyhalogenated aliphatic aldehydes such as—acetaldehyde, propionaldehyde, butyraldehyde, caproaldehyde, acrolein, crotonaldehyde, ethyl butyraldehyde, ethyl propyl aldehyde, 2-ethyl hexanol, chloral, butyl chloral, heptaldehyde, etc.

VI. Polyhalogenated aromatic aldehydes such as—benzaldehyde, paratoluic aldehyde, cinnamaldehyde, salicylaldehyde, naphthaldehyde, vanillin, phenylacetraldehyde, laurylbenzaldehyde, etc.

VII. Other types of polyhalogenated aldehydes such as—glycol-aldehydes, methoxy furfural benzaldehyde, etc.

The halogen atoms attached to the carbonyl compounds may be chlorine which is preferred or bromine and the like or the mixtures. Halogenation of these compounds may be carried out in any suitable manner. Preferred carbonyl com-

pounds are chloral, butyl chloral, bromal, polychlorobutanol, polyclorpentanol, trichlorobenzophenone, polychlorocyclohexanone, polychlorpalmitone, polychlorstearone, polychlormethyl isobutyl ketone and the like.

The thiol, selenol and/or telurol organic compounds used to react with the polyhalogenated organic carbonyl compounds may be any organic compound containing the SH, SeH and/or TeH radicals and may include:

I. Aliphatic compounds containing substitute radical of SH, SeH and/or TeH of—methyl, ethyl, normal propyl, isopropyl, normal and isobutyl, secondary butyl, tertiary butyl, normal amyl, isoamyl, tertiary amyl, tertiary octyl, tertiary decyl, tertiary dodecyl, tertiary hexadecyl, hexyl, octyl, lauryl thiols or mercaptans, selenols, telurols and the like.

II. Aromatic compounds containing SH, SeH and/or TeH groups linked directly to the aromatic nucleus or aromatic compounds in which the aromatic nucleus is separated from the SH, SeH or TeH groups by intervening carbon atoms in the chain such as—phenyl, chlorophenyl, tolyl, xylyl, naphthyl, benzyl, phenylethyl, tolylpropyl mercaptans or thiols, selenols, telurols and the like.

III. Unsaturated alkyl and aryl thiol, selenol and telurol compounds such as—allyl, crotyl, methallyl, cinnamyl thiols, selenols and/or telurols and the like.

The above thiol, selenol, and telurol containing compounds may be made by any suitable means or obtained from any suitable source. Thus mercaptans may be extracted by a caustic alkali treatment of petroleum hydrocarbon fractions. Also these compounds may contain various substituent groups such as halogen, acid groups and the like.

The reaction between the halogen containing organic carbonyl compounds and the thiol, selenol and/or telurol compounds may be carried out in aqueous acid medium with the aid of slightly elevated temperature. The resulting halogen bearing acetal derivative having the general formula as in column 3 may be recovered from the solution by suitable means such as by crystallization and the like. The reaction product thus formed is of sufficient purity so that it can be used in lubricants without further purification, such as recrystallization or the like.

To more clearly illustrate the present invention, the following examples are presented. It is to be understood however that various modifications can be resorted to without departing from the spirit of the invention.

*Example I*

Approximately one mole of chloral was dissolved in about 2000 parts by volume of water and about 50 parts by volume of concentrated hydrochloric acid was slowly added to the mixture with constant stirring. To this mixture approximately 2 moles of ethyl mercaptan was added and the mixture agitated and gently heated to about 60° C. The polychlorthioacetal was deposited out of the solution as a crystalline condensation product and recovered therefrom. The faint odor of the parent mercaptan may be removed by recrystallization of the reaction product. The product having the appearance of white needles had a melting point of about 61° C. and was readily soluble in mineral lubricating oil.

*Example II*

Approximately one mole of chloral hydrate was dissolved in about 2000 parts by volume of water and about 50 parts by volume of concentrated hydrochloric acid was slowly added to the mixture with constant stirring. To this mixture approximately 2 moles of ethyl mercaptan was added and the mixture agitated and gently heated to about 60° C. The polychlorthioacetal was deposited out of the solution as a crystalline condensation product and recovered therefrom. The faint odor of the parent mercaptan may be removed by recrystallization of the reaction product. The product having the appearance of white needles had a melting point of about 61° C. and was readily soluble in mineral lubricating oil.

*Example III*

Approximately one mole of chloral was dissolved in about 2000 parts by volume of water and about 50 parts by volume of concentrated hydrochloric acid was slowly added to the mixture with constant stirring. To this mixture approximately 2 moles of normal butyl mercaptan was added and the mixture agitated and gently heated to about 60° C. The polychlorthioacetal was deposited out of the solution as a crystalline condensation product and recovered therefrom. The faint odor of the parent mercaptan may be removed by recrystallization of the reaction product. The product having the appearance of white needles had a melting point of about 55° C. and was readily soluble in mineral lubricating oil.

*Example IV*

Approximately one mole of chloral was dissolved in about 2000 parts by volume of water and about 50 parts by volume of concentrated hydrochloric acid was slowly added to the mixture with constant stirring. To this mixture approximately 2 moles of isobutyl mercaptan was added and the mixture agitated and gently heated to about 60° C. The polychlorthioacetal was deposited out of the solution as a crystalline condensation product and recovered therefrom. The faint odor of the parent mercaptan may be removed by recrystallization of the reaction product. The product having the appearance of white needles had a melting point of about 46° C. and was readily soluble in mineral lubricating oil.

*Example V*

Approximately one mole of chloral was dissolved in about 2000 parts by volume of water and about 50 parts by volume of concentrated hydrochloric acid was slowly added to the mixture with constant stirring. To this mixture approximately 2 moles of phenyl mercaptan was added and the mixture agitated and gently heated to about 60° C. The polychlorthioacetal was deposited out of the solution as a crystalline condensation product and recovered therefrom. The faint odor of the parent mercaptan may be removed by recrystallization of the reaction product. The product having the appearance of white needles had a melting point of about 82° C. and was readily soluble in mineral lubricating oil.

*Example VI*

Approximately one mole of chloral was dissolved in about 2000 parts by volume of water and about 50 parts by volume of concentrated hydrochloric acid was slowly added to the mixture with constant stirring. To this mixture approximately 2 moles of benzyl mercaptan was added and the mixture agitated and gently heated to about 60° C. The polychlorthioacetal was deposited out of the solution as a crystalline condensation product and recovered therefrom. The faint odor of the parent mercaptan may be removed by recrystallization of the reaction product. The product having the appearance of white needles had a melting point of about 80° C. and was readily soluble in mineral lubricating oil.

All of the reaction products as prepared as disclosed in Examples I to VI when added in amounts of less than 1% by weight and preferably around about 0.25% by weight in a 150 Pennsylvania Neutral oil and subjected to a Four Ball Machine test as described in Engineering, July 14, 1933, gave excellent extreme pressure results.

| Per Cent Additive in Mineral Oil                     | Mean Wear Diameter (mm.) at various loads |      |      |      |      |      | Coefficient of friction at various loads |    |      |      |      |      |
|------------------------------------------------------|-------------------------------------------|------|------|------|------|------|------------------------------------------|----|------|------|------|------|
|                                                      | 80                                        | 100  | 140  | 200  | 260  | 300  | 7                                        | 15 | 80   | 100  | 260  | 300  |
| None                                                 | 3.14                                      | Weld | —    | —    | —    | —    | 0.127                                    | —  | —    | —    | —    | —    |
| 1% of Reaction Product of Example III in Mineral oil | 0.65                                      | 1.50 | 2.00 | 2.20 | —    | —    | —                                        | —  | 0.05 | 0.07 | —    | —    |
| 1% of Reaction Product of Example IV in Mineral oil  | 0.40                                      | 0.70 | 1.68 | 2.00 | 2.36 | —    | —                                        | —  | 0.05 | 0.05 | 0.08 | —    |
| 1% of Reaction Product of Example V in Mineral oil   | 0.04                                      | 0.70 | 1.40 | 1.60 | 2.05 | 2.25 | —                                        | —  | 0.05 | 0.05 | 0.08 | 0.08 |

Other reaction products of this invention which are preferred as additives for lubricants are:

Chlorobutanal-ethyl mercaptan  
Chlorobutanal-phenyl mercaptan  
Chlorobutanal-cetyl mercaptan  
Chlorobutanal-ethyl selenol  
Chloropentanal-ethyl mercaptan  
Chloropentanal-butyl mercaptan  
Chloropentanal-benzyl mercaptan  
Chloropentanal-phenyl mercaptan  
Chloropentanal-ethyl selenol  
Chlorocyclobutanone-ethyl mercaptan  
Chlorocyclobutanone-butyl mercaptan  
Chlorocyclobutanone-phenyl mercaptan  
Chlorocyclobutyl methyl ketone-ethyl mercaptan  
Chlorocyclobutyl methyl ketone-butyl mercaptan  
Chlorocyclobutyl methyl ketone-phenyl mercaptan  
Chlorostearone-ethyl mercaptan  
Chlorostearone-phenyl mercaptan  
Chlorostearone-benzyl mercaptan  
Butyl chloral-ethyl mercaptan

Reaction products of this invention are highly effective extreme pressure agents for various types of lubricants and generally need not be used in amounts greater than 1% by weight. However, concentrations of as high as from 1 to 10% may be used under certain conditions of lubrication. For other purposes, additives of this invention need only be incorporated, for example in a mineral lubricating oil or grease, in amounts of between about 0.25 and 0.5% to exert a marked improvement in the behavior of a lubricant in service involving extreme pressure.

The base lubricant or oil may be a hydrocarbon oil of the paraffins, naphthenic or asphaltic type of wide viscosity range. The oils may be refined or treated by any desirable means so as to obtain fractions suitable for specific lubricating needs. Generally SAE 10 to 50 or even higher oils may be used. In addition to natural hydrocarbon oils, natural occurring fatty materials such as fixed fatty oils and mixtures of such oils with hydrocarbon oils may be used. Also synthetic type lubricants such as polymerized olefins, copolymers of alkylene glycols and alkylene oxides, organic esters, e. g. 2-ethyl hexyl sebacate, dioctyl phthalate, trioctyl phosphate; polymeric tetrahydrofuran, polyalkyl silicon polymers and the like may be used as well as mixtures of synthetic and natural lubricants. Also reaction products of this invention may be added to fuels, wax products, cutting compositions and the like.

Because of its synergistic effect the reaction product of this invention can be combined with other additives in lubricants, such as, blooming agents, pour point depressants or viscosity improvers, extreme pressure agents, antifoaming agents and the like. Among the specific additives which can be used are oil-soluble detergents which include oil-soluble salts of various bases with detergent forming acids. Such bases include metal as well as organic bases. Metallic bases include those of the alkali metals, Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

Examples of detergent forming acids are the various fatty acids of, say, 10 to 30 carbon atoms, wool fat acids, paraffin wax acids (produced by oxidation of paraffin wax) chlorinated fatty acids, rosin acids, aromatic carboxylic acids including aromatic fatty acids, aromatic hydroxy fatty

7  
8  
acids, paraffin wax benzoic acids, various alkyl salicylic acids, phthalic acid mono-esters, aromatic keto acids, aromatic ether acids, diphenols as di-(alkylphenol) sulfides and disulfides, methylene bis alkylphenols; sulfonic acids such as may be produced by treatment of alkyl aryl hydrocarbons or high boiling petroleum oils with sulfuric acid; sulfuric acid mono-esters; phosphoric, arsenic and antimony acid mono and diesters, 10 including the corresponding thio phosphoric, arsenic and antimony acids; phosphonic and arsenic acids and the like.

Additional detergents are the alkaline earth phosphate diesters, including the thiophosphate diester; the alkaline earth diphenolates, specifically the calcium and barium salts of diphenol mono and poly sulfides.

Non-metallic detergents include compounds such as the phosphatides such as lecithin and cephalin, certain fatty oils as rapeseed oils, volatilized fatty or mineral oils and the like.

An excellent metallic detergent for the present purpose is the calcium salt of oil-soluble petroleum sulfonic acids. This may be present advantageously in the amount of about 0.025% to 0.2% sulfate ash. Also alkaline metal salts of alkyl phenol-aldehyde condensation reaction products are excellent detergents.

Antioxidants comprise several types, for example, alkyl phenols such as 2,4,6 trimethyl phenol, penta methyl-phenol, 2,4 dimethyl-6-tertiary-butyl phenol, 2,4-dimethyl-6-octyl phenol, 2,6-di-tertiary-butyl-4-methyl-phenol, 2,4,6 tritertiary-butyl phenol and the like; amino phenols as benzyl amino phenols; amines such as dibutyl-phenylene diamine, diphenyl amine, phenyl-beta-naphthylamine, phenyl-alpha-naphthylamine, dinaphthyl amine.

Corrosion inhibitors or anti-rusting compounds 40 may also be present, such as dicarboxylic acids of 16 and more carbon atoms; alkali metal and alkaline earth salts of sulfonic acids and fatty acids; organic compounds containing an acidic radical in close proximity to a nitrile, nitro or nitroso group (e. g. alpha cyano stearic acid).

Extreme pressure agents which may be used comprise: esters of phosphorus acids such as tri-aryl, alkyl hydroxy aryl, or aralkyl phosphates, thiophosphates or phosphites and the like; neutral aromatic sulfur compounds of relatively high boiling temperatures such as diaryl sulfides, diaryl disulfides, alkyl aryl disulfides, e. g. diphenyl sulfide, diphenol sulfide, dicrosol sulfide, dixylenol sulfide, methyl butyl diphenol sulfide, dibenzyl sulfide, corresponding di- and tri-sulfides, and the like; sulfurized fatty oils or esters of fatty acids and monohydric alcohols, e. g. sperm oil, jojoba oil, etc.; in which the sulfur is strongly bonded; sulfurized long chain olefins such as may be obtained by dehydrogenation or cracking of wax; sulfurized phosphorized fatty oils or acids, phosphorus acid esters having sulfurized organic radicals, such as esters of phosphoric or phosphorus acids with sulfurized hydroxy fatty acids; chlorinated hydrocarbons, such as chlorinated paraffin, aromatic hydrocarbons, terpenes, mineral lubricating oil, etc.; or chlorinated esters of fatty acids containing the chlorine in position other than alpha position.

Additional ingredients may comprise oil-soluble urea or thiourea derivatives, e. g. urethanes, aliphonates, carbazides, carbazones, etc.; polyisobutylene polymers, unsaturated polymerized esters of fatty acids and monohydric alcohols and other high molecular weight oil-soluble compounds.

Depending upon the additive used and conditions under which it is used, the amount of additive used may vary from 0.1 to 2% or higher. However, substantial improvement is obtained by using amounts ranging from 0.1 to 0.5% in combination with polyhalogen containing organic carbonyl compound and organic thiol, selenol and/or telurol compound reaction products of this invention.

The novel reaction products of this invention, in addition to being excellent lubricating oil improving agents, are potent oxidation inhibitors for fuels, natural and synthetic rubber, wax coating compositions and other organic materials.

It is to be understood that while the features of the invention have been described and illustrated in connection with certain specific examples, the invention, however, is not to be limited thereto or otherwise restricted, except by the prior art and the scope of the appended claims.

I claim as my invention:

1. A lubricating composition consisting essentially of a major amount of a hydrocarbon oil and a minor amount of less than 1% sufficient to impart extreme pressure properties to said lubricant of trichloromethyl di(thiaethyl) methane.

2. A lubricating composition consisting essentially of a major amount of a hydrocarbon oil and a minor amount of less than 1% sufficient to impart extreme pressure properties to said lubricant of trichloromethyl di(thiabenzyl) methane.

3. A lubricating composition consisting essentially of a major amount of a hydrocarbon oil and a minor amount of less than 1% sufficient to impart extreme pressure properties to said lubricant of trichloromethyl di(thiaphenyl) methane.

4. A lubricating composition consisting essentially of a major amount of a hydrocarbon oil and a minor amount of less than 1% sufficient to impart extreme pressure properties to said lubricant of a polychlorinated acetal having the general configuration



wherein X is an element of the group consisting of S, Se and Te, A is an organic radical having a plurality of chlorine atoms and each R1 is an independently selected organic radical.

5. A lubricating composition comprising a lubricating oil and a minor amount, but sufficient to impart extreme pressure properties to said lubricant and not exceeding 10% by weight, of a polychlorinated acetal having the general configuration



wherein A is an organic radical having a plurality of chlorine atoms and each R1 is an independently selected organic radical.

6. A lubricating composition comprising a lubricating oil and a minor amount, but sufficient to impart extreme pressure properties to said lubricant and not exceeding 10% by weight, of trichloromethyl di(thiaalkyl) methane.

7. A lubricating composition comprising a lubricating oil and a minor amount, but sufficient to impart extreme pressure properties to said

lubricant and not exceeding 10% by weight, of trichloromethyl di(thiaaryl) methane.

8. A lubricating composition comprising a lubricating oil and a minor amount, but sufficient to impart extreme pressure properties to said lubricant and not exceeding 10% by weight, of trichloromethyl di(thiaaralkyl) methane.

9. A lubricating composition comprising a lubricating oil and a minor amount, but sufficient to impart extreme pressure properties to said lubricant and not exceeding 10% by weight, of trichloromethyl di(thiaethyl) methane.

10. A lubricating composition comprising a lubricating oil and a minor amount, but sufficient to impart extreme pressure properties to said lubricant and not exceeding 10% by weight, of trichloromethyl di(thiabenzyl) methane.

11. A lubricating composition comprising a lubricating oil and a minor amount, but sufficient to impart extreme pressure properties to said lubricant and not exceeding 10% by weight, of trichloromethyl di(thiaphenyl) methane.

12. A lubricating composition comprising a hydrocarbon oil and a minor amount, but sufficient to impart extreme pressure properties to said lubricant and not exceeding 10% by weight, of a polyhalogenated acetal having the general configuration



wherein X is an element of the group consisting of S, Se and Te, A is an organic radical having a plurality of halogen atoms and each R1 is an independently selected organic radical.

13. A lubricating composition comprising a hydrocarbon oil and a minor amount, but sufficient to impart extreme pressure properties to said lubricant and not exceeding 10% by weight, of a polyhalogenated acetal having the general configuration



wherein X is an element of the group consisting of S, Se and Te, A is an aliphatic organic radical having a plurality of halogen atoms and each R1 is an independently selected aliphatic organic radical.

14. A lubricating composition comprising a hydrocarbon oil and a minor amount, but sufficient to impart extreme pressure properties to said lubricant and not exceeding 10% by weight, of a polyhalogenated acetal having the general configuration



wherein X is an element of the group consisting of S, Se and Te, A is an aromatic organic radical having a plurality of halogen atoms and each R1 is an independently selected aromatic organic radical.

15. A lubricating composition comprising a hydrocarbon oil and a minor amount, but sufficient to impart extreme pressure properties to said lubricant and not exceeding 10% by weight

of a polyhalogenated acetal having the general configuration



wherein X is an element of the group consisting of S, Se and Te, A is an aralkyl organic radical having a plurality of halogen atoms and each R1 is an independently selected aralkyl organic radical.

WILLIAM DAVEY.

REFERENCES CITED

The following references are of record in the file of this patent:

UNITED STATES PATENTS

|   | Number    | Name           | Date          |
|---|-----------|----------------|---------------|
| 5 | 2,223,693 | Martin         | Dec. 3, 1940  |
|   | 2,353,170 | Lincoln et al. | July 11, 1944 |
|   | 2,422,341 | Crouch         | June 17, 1947 |
|   | 2,444,525 | Pavlic         | July 6, 1948  |

FOREIGN PATENTS

|    | Number  | Country       | Date          |
|----|---------|---------------|---------------|
| 10 | 514,535 | Great Britain | Nov. 10, 1939 |

OTHER REFERENCES

|    |        |                                                |
|----|--------|------------------------------------------------|
| 15 | Number | Iowa State College Journal Science, 16, 99-102 |
|    |        | (1941).                                        |